

1

3,249,545

LUBRICATING COMPOSITION CONTAINING  
NON-ASH FORMING ADDITIVES

Henricus G. P. van der Voort, Maurits Krukziener, Jan B. Baudoux, and Hendrik van Oosten, Amsterdam, Netherlands, assignors to Shell Oil Company, New York, N.Y., a corporation of Delaware  
No Drawing. Filed Oct. 12, 1962, Ser. No. 230,279  
Claims priority, application Netherlands, Mar. 23, 1962, 276,299

3 Claims. (Cl. 252—49.8)

This invention relates to improved lubricating oil compositions possessing multifunctional properties. More particularly, the invention relates to mineral lubricating oils useful in the lubrication of engines operating over wide temperature ranges and under extreme pressures and other adverse conditions.

It is known that lubricating oils containing certain metallic salts or soaps such as metal sulfonates possess good dispersing and detergent properties. Such lubricants, however, tend to form metallic deposits in engine parts which interfere with the effective operation of the engine. In the lubrication of combustion engines with a lubricant containing a metallic additive, the ash deposits formed in the combustion chamber and on the valves causes engine operating difficulties as, for instance premature ignition of the air/fuel mixture, etc. Because of these deficiencies attributable to ash-containing additives, ashless additives have been developed such as non-ash forming basic and essentially neutral nitrogen-containing dispersants of high molecular weight such as copolymers of polymerizable amines or amides with long-chain acrylate esters. Ashless additives of this type are available commercially under the trade names of LOA-564 or 565, Acryloid 315X, 917 or 966 and described in U.S. Patent 2,737,469 and Belgian Patent 550,422 respectively. These non-ash forming polymeric compounds are good detergents but under extreme pressure conditions lack stability and wear inhibiting properties and are also ineffective as sludge and corrosion inhibitors. Attempts to overcome these deficiencies by modification of these polymers or by use of auxiliary additives in combination with these polymers has met with little success. Thus modifying polymers by introducing certain groups tends often to destroy or reduce the original desirable properties which the polymers possess. In certain cases where auxiliary additives appear to be promising stabilizers and wear inhibitors they are usually metal-containing compounds such as metal sulfonates or metal carboxylates. For reasons stated, compounds of this type are to be avoided and because of their tendency to complex with the polymer and form sludge.

It is an object of the present invention to provide an improved non-ash forming lubricating oil composition. It is another object of the invention to provide an improved detergent lubricant possessing good stability and anti-wear properties. Still another object of the invention is to provide a corrosion and sludge resistant non-ash containing lubricating oil composition. Other objects will become apparent during the following description of the invention.

Now in accordance with the present invention, it has been found that stability, as well as sludge, wear and corrosion inhibition can be imparted to lubricating oil composition by incorporating therein small amount of (1) an oil-soluble detergent copolymer of (A) an ester of an unsaturated monocarboxylic acid and a monohydric aliphatic alcohol having 4-30 carbon atoms and (B) an ester of an unsaturated aliphatic carboxylic acid and a polyhydric alcohol and (2) certain oil-soluble bisphenols which normally are known for the anti-oxidant properties but in combination with detergent copolymers of the present invention functions as a wear and corrosion inhibitor. The

2

detergent copolymers per se also lack anti-oxidant and wear inhibiting properties and primarily are added to lubricants as detergent-dispersant additives. Therefore, the additive combination imparts to base lubricants, unexpected unusual properties.

The copolymeric additives (1) are copolymers with ester groups derived from monomeric esters of unsaturated monocarboxylic acids, such as acrylic acid, methacrylic acid, crotonic acid, tiglic acid and angelic acid, and monohydric alcohols, such as the octanols, lauryl alcohol and stearyl alcohol, and (2) ester groups derived from monomeric esters of unsaturated carboxylic acids as mentioned hereinbefore, and polyhydric alcohols, such as glycols, trivalent alcohols, such as glycerine and higher alcohols, such as erythritol, pentaerythritol, mannitol and the like.

Also suitable are copolymers with ester groups derived from di-esters of the alcohols mentioned hereinbefore, and unsaturated dicarboxylic acids, such as maleic acid, fumaric acid, mesaconic acid, citraconic acid and the like. Copolymers with ester groups derived from the aforesaid alcohols and both an unsaturated monocarboxylic acid and an unsaturated dicarboxylic acid, for instance a copolymer derived from mixtures of methacrylate esters and di-esters of maleic acid also can be used in composition of the present invention.

In the preparation of the copolymers of the present invention unsaturated monocarboxylic acids, e.g. methacrylic and acrylic acids are preferred and in the case of the polymerizable ester of a polyhydric alcohol unsaturates esters of ethylene glycols are preferred.

The copolymeric esters of groups (A) and (B) can be derived from mixtures of esters from each groups (A) and (B). As for example, copolymers can be prepared by copolymerization of an ester mixture obtained from an unsaturated acid and an alcohol mixture such as coconut fatty alcohols, with esters obtained from an unsaturated acid and a polyhydric alcohol or mixtures of polyhydric alcohols.

The detergent-dispersant copolymers of the present invention can be modified and viscosity index and pour depressant properties imparted thereto by forming cross-linked polymers therefrom by copolymerizing the copolymers of the present invention with diolefins compound such as a dimethacrylate ester of ethylene glycol, divinyl esters, e.g. divinyl adipate and the like fully described in Henricus G. P. van der Voort's copending patent application Serial No. 230,278 filed Oct. 12, 1962.

Illustrative examples of copolymers of the present invention are as follows:

## COPOLYMER I

Copolymer of stearyl methacrylate, lauryl methacrylate and 2-hydroxyethyl methacrylate in the molar ratio of 5:5:3. The intrinsic viscosity of the copolymer, determined at 98.9° C. in an extracted paraffinic lubricating oil distillate, was 0.65 dl./g.

## COPOLYMER II

Copolymer of stearyl methacrylate, lauryl methacrylate, 2-hydroxyethyl methacrylate and the dimethacrylate ester of ethylene glycol in the molar ratio of 5:5:3:0.03. The intrinsic viscosity of the copolymer, determined at 98.9° C. in an extracted paraffinic lubricating oil distillate, was 0.65 dl./g.

The other additive which is used in combination with the essential detergent copolymeric additive (1) of this invention is (2) an alkylated bisphenol having the formula



wherein R' is a hydrocarbyl radical, preferably a C<sub>1-8</sub> alkyl radical, y is an integer of 1 to 4, preferably 1 or 2, X stands for —S—, —S—S—, Se, —S—CH<sub>2</sub>—,



—CH<sub>2</sub>—O—CH<sub>2</sub>—, —CHR—, CR<sub>2</sub>—, —(CH<sub>2</sub>)<sub>m</sub>—, —NH—, —O—, and wherein R stands for methyl or ethyl and m stands for an integer from 1 to 3. The preferred alkylated bisphenols are those having a sulfur bridge or a methylene bridge.

The alkylated bisphenols may contain from 1 to 8 alkyl groups, but preferably they contain from 2 to 6 alkyl groups. Alkylated bisphenols having 4 alkyl groups are particularly preferred. Each of the alkyl groups may contain from 1 to 10 carbon atoms, preferably 2 to 6 carbon atoms and especially 4 carbon atoms. Furthermore, the alkyl groups contained by any particular bisphenol may be the same or different and may also be primary, secondary, or tertiary alkyl groups. Bisphenols containing at least one tertiary alkyl group are particularly preferred.

As examples of the alkylated bisphenols which may be used according to the invention there are mentioned

bis(3-ethyl-4-hydroxyphenyl)disulfide,  
bis(3-methyl-4-propyl-5-hydroxyphenyl)disulfide,  
bis(2-isopropyl-3-butyl-5-hydroxyphenyl)selenide,  
2:2'-diethyl-3-tertiary butyl-4,4'-dihydroxy diphenyl selenide,  
bis 1.2(2:6-di-tertiary butyl-4-hydroxyphenyl)thiaethane,  
bis 1.2(2:5-di-isopropyl-3-hydroxyphenyl)thiaethane,  
bis(3:5-di-tertiary butyl-4-hydroxyphenyl)sulfide,  
2:4-di-isobutyl-3-hydroxybenzyl-2':4'-dipropyl-3'-hydroxy-benzyl sulfide,  
bis 1.2(3-octyl-5-tertiary butyl-4-hydroxyphenyl)ethane,  
bis 1.1(2:6-di-isopropyl-4-hydroxyphenyl)ethane,  
1.2-bis(2:4-di-tertiary pentyl-3-hydroxyphenyl)propane,  
bis 2.2(4:5-di-tertiary butyl-2-hydroxyphenyl)propane,  
bis(2-tertiary butyl-5-isopentyl-4-hydroxyphenyl)amine,  
bis(3:5-dibutyl-4-hydroxyphenyl)ether,  
bis(2:6-dipropyl-4-hydroxyphenyl)ether.

Examples of alkylated bis-phenols having a sulfur bridge are

bis(2:5-dipentyl-4-hydroxyphenyl)sulfide,  
bis(2:5-dihexyl-3-hydroxyphenyl)sulfide,  
bis(2-methyl-5-tertiary butyl-4-hydroxyphenyl)sulfide,  
bis(2-methyl-5-tertiary butyl-6-hydroxyphenyl)sulfide  
and particularly bis(3-tertiary butyl-5-methyl-2-hydroxyphenyl)sulfide.

Examples of alkylated bisphenols having a methylene bridge are

bis(2:3-di-tertiary butyl-4-hydroxyphenyl)methane,  
bis(2:5-di-tertiary butyl-4-hydroxyphenyl)methane,  
bis(2:6-di-tertiary butyl-4-hydroxyphenyl)methane,  
bis(3:5-di-tertiary octyl-4-hydroxyphenyl)methane,  
bis(3-tertiary butyl-5-tertiary octyl-4-hydroxyphenyl)methane,  
and especially bis(3:5-di-tertiary butyl-4-hydroxyphenyl)methane,  
(3,5-difert-butyl-3',5'-dimethyl-4:4'-dihydroxydiphenyl)methane,  
(3,5-difert-butyl-3',5'-diisopropyl-4:4'-dihydroxydiphenyl)methane,  
3,5,5'-difert-butyl-2,4'-dihydroxydiphenyl)methane.

The alkylated bisphenol may be prepared by any of the methods known in the art of bisphenols as starting materials and condensing them together by any of the established methods.

The lubricating oil compositions according to the invention may be further improved by addition of small amounts of other additives which are metal-free organic phosphorus-containing compounds such as alkyl, cycloalkyl, alkaryl, aralkyl, and aryl phosphites, phosphates,

phosphonates, and their thio- derivatives, such as C<sub>3-18</sub> alkyl phosphites, e.g. di and tributyl, octyl, lauryl, stearyl, cyclohexyl, benzyl, cresyl, phenyl phosphites or phosphates, as well as their thio-derivatives; P<sub>2</sub>S<sub>5</sub>-terpene reaction product; organo phosphonates, e.g. dibutyl methanephosphonate, dibutyl trichloromethanephosphonate, dibutyl monochloromethanephosphonate, dibutyl chlorobenzenephosphonate, dibutyl monochloromethanephosphonate, dibutyl chlorobenzenephosphonate and the like. The esters of pentavalent phosphorus acids such as diphenyl, dicesyl, triphenyl, tricesyl, triauryl and tri-stearyl phosphate, P<sub>2</sub>S<sub>5</sub>-terpene reaction products and mixtures thereof are preferred.

The concentrations of the various components of the lubricant compositions may vary within wide limits. For instance, the copolymers can be used in concentrations varying from 0.1 to 10% by weight, the bisphenol, in concentrations varying from 0.01 to 5% by weight and the phosphorus-containing compound in concentrations varying, for instance, from 0.01 to 5% by weight. Preferably, lubricant compositions are prepared with a content of copolymers varying from 0.5 to 2% by weight, a content of bisphenol varying from 0.5 to 2% by weight and, if a phosphate, e.g. an aryl phosphate is used, it may vary from 0.5 to 2% by weight.

Lubricants of divergent nature can be used for preparing the lubricant compositions according to the invention. In the first place mineral lubricating oils of varying viscosities may be mentioned. Synthetic lubricating oils are, however, also suitable, as well as lubricating oils containing fatty oils. Lubricating greases can also be applied.

For preparing the lubricant compositions according to the invention preferably a mineral lubricating oil is used.

In preparing the lubricant composition it may be an advantage first to prepare a concentrated solution of the copolymer, the bisphenol and, if used, the phosphate, in a solvent or a lubricant and subsequently, for instance elsewhere, to dilute the concentrated solution with a lubricant and to remove by distillation under reduced pressure or by steam distillation. The following are illustrative compositions of the present invention:

| Composition A                                                                                      |             |
|----------------------------------------------------------------------------------------------------|-------------|
| 45                                                                                                 | Percent wt. |
| Base oil: extracted paraffinic lubricating oil distillate with a viscosity of 6.82 cs. at 98.9° C. | 97.75       |
| Copolymer I                                                                                        | 1.5         |
| Bis(3,5-di-tert-butyl-4-hydroxyphenyl)methane                                                      | 0.75        |

| Composition B                                 |       |
|-----------------------------------------------|-------|
| Base oil: as in A                             | 97.75 |
| Copolymer II                                  | 1.5   |
| Bis(3,5-di-tert-butyl-4-hydroxyphenyl)methane | 0.75  |

| Composition C                                                                                     |       |
|---------------------------------------------------------------------------------------------------|-------|
| Base oil: extracted paraffinic lubricating oil distillate with a viscosity of 4.5 cs. at 98.9° C. | 97.75 |
| Copolymer I                                                                                       | 1.5   |
| Bis(3,5-di-tert-butyl-4-hydroxyphenyl)methane                                                     | 0.75  |

| Composition D     |      |
|-------------------|------|
| Base oil: as in C | 98.5 |
| Copolymer I       | 1.5  |

| Composition E                                 |       |
|-----------------------------------------------|-------|
| Base oil: as in C                             | 99.25 |
| Bis(3,5-di-tert-butyl-4-hydroxyphenyl)methane | 0.75  |

| Composition F                                 |       |
|-----------------------------------------------|-------|
| Base oil: as in C                             | 96.75 |
| Copolymer I                                   | 1.5   |
| Bis(3,5-di-tert-butyl-4-hydroxyphenyl)methane | 0.75  |
| Triphenyl phosphate                           | 1.0   |

The improvement which the additive combination of the present invention impart to lubricating oils is apparent from the test data shown below.

## VISCOSEITY INDEX

The viscosity indices of compositions A and B were determined according to Dean and Davis (A. Bondi, Physical Chemistry of Lubricating Oils, 1951, pp. 50 ff.) and the results of these measurements are given in Table I.

TABLE I

|               |         |
|---------------|---------|
| Composition A | 138     |
| Composition B | 144     |
| Base oil A    | 100-110 |

## ANTI-WEAR EFFECT

The anti-wear effect at high load was determined in tests in which the valve system of a four-cylinder Opel engine was lubricated with lubricating oil compositions according to the invention and also in tests in the four-ball top.

## OPEL TESTS

After removal of the pistons and connecting rods the engine was powered by an electric motor. The tension of the loaded valve spring of about 60 kg. was increased to about 85 kg. by inserting a metal disc between spring and spring seat. The speed of the crankshaft was 2920 r.p.m., hence that of the camshaft 1460 r.p.m. The oil temperature was 90 C.; the amount of oil put into the crankcase was 1.25 kg.

The test was continued until the valve tappets became useless owing to particles of metal crumbling away from the camloaded surface. The results of these tests are recorded in Table II.

TABLE II

| Oil composition | Test No. | Duration of test, hours | Number of damaged valve tappets |
|-----------------|----------|-------------------------|---------------------------------|
| C               | 17       | 85                      | none                            |
| D               | 18       | 82.5                    | 3                               |
| E               | 21       | 16.5                    | 7                               |

## FOUR-BALL TOP

The anti-wear effect at heavy load was determined in the four-ball top at room temperature and at 130° C. The four-ball top is described in "Four-Ball Top for testing boundary lubricating properties under high mean pressures," G. D. Boerlage and H. Blok, Engineering, Vol. 144, p. 1 (1937).

The results are shown in Table III.

6  
TABLE III

|                           | Diameter of wearing surface, mm. |         |
|---------------------------|----------------------------------|---------|
|                           | Room temperature                 | 130° C. |
| Base oil of composition C | 0.34                             | 0.40    |
| Composition C             | 0.28                             | 0.38    |
| Composition F             | 0.14                             | 0.18    |

Other additives may also be incorporated into the lubricating composition according to the invention, for example anti-scuffing agents; anti-foaming agents, e.g. silicone polymers; viscosity index improvers, for example polymeric acrylic esters; extreme pressure additive, for example dibenzyl disulfide; rust inhibitors, for example sorbitan monooleate or butyl stearate; oiliness agents, for example acidless tallow, oleic acid and the like.

We claim as our invention:

1. A mineral lubricating oil composition comprising a major amount of mineral lubricating oil and from about 0.1% to about 10% of an oil-soluble copolymer of a mixture of dissimilar C<sub>12-18</sub> alkyl methacrylates and 2-hydroxyethyl methacrylate, the copolymer having an intrinsic viscosity of around 0.65 dl./g. and from about 0.5% to about 2% of bis(3,5-ditertiarybutyl-4-hydroxyphenyl)methane.
2. A mineral lubricating oil composition comprising a major amount of mineral lubricating oil and from about 0.1% to about 10% of an oil-soluble copolymer of stearyl methacrylate, lauryl methacrylate and 2-hydroxyethyl methacrylate having an intrinsic viscosity of about 0.65 dl./g. and from about 0.5% to about 2% of bis(3,5-ditertiarybutyl-4-hydroxyphenyl)methane.
3. The composition of claim 2 containing from about 0.5% to about 2% of tricresyl phosphate.

## References Cited by the Examiner

## UNITED STATES PATENTS

|           |         |                  |            |
|-----------|---------|------------------|------------|
| 2,157,873 | 5/1939  | Van Peski et al. | 252-49.8 X |
| 2,636,861 | 4/1953  | Watson           | 252-49.8 X |
| 2,681,987 | 6/1954  | Frazier          | 260-78.5   |
| 2,892,819 | 6/1959  | Stewart et al.   | 252-56     |
| 2,944,086 | 7/1960  | Coffield         | 252-52     |
| 2,998,414 | 8/1961  | West et al.      | 252-56     |
| 3,001,942 | 9/1961  | Mulvany et al.   | 252-56     |
| 3,002,959 | 10/1961 | Hicks            | 260-78.5 X |
| 3,028,367 | 4/1962  | O'Brien          | 260-86.1 X |
| 3,056,764 | 10/1962 | Graham et al.    | 260-78.5 X |
| 3,060,226 | 10/1962 | Munn             | 260-86.1 X |

DANIEL E. WYMAN, Primary Examiner.

L. G. XIARHOS, Assistant Examiner.